

J. H. PAYNE,  
ELECTRICAL RESISTANCE,  
APPLICATION FILED NOV. 21, 1917.

1,291,106.

Patented Jan. 14, 1919.

Fig.1.



Fig.2.



Fig.3.



Inventor:  
John H. Payne,  
by *Almon G. Davis*  
His Attorney.

# UNITED STATES PATENT OFFICE.

JOHN H. PAYNE, OF BALLSTON SPA, NEW YORK, ASSIGNOR TO GENERAL ELECTRIC COMPANY, A CORPORATION OF NEW YORK.

## ELECTRICAL RESISTANCE.

1,291,106.

Specification of Letters Patent. Patented Jan. 14, 1919.

Application filed November 21, 1917. Serial No. 203,071.

*To all whom it may concern:*

Be it known that I, JOHN H. PAYNE, a citizen of the United States, residing at Ballston Spa, in the county of Saratoga, 5 State of New York, have invented certain new and useful Improvements in Electrical Resistances, of which the following is a specification.

The present invention comprises a novel 10 resistance unit which is particularly suitable for use in receiving systems for wireless telegraphy, particularly in amplifying systems or and instances when a unit of constant known high resistance is desired.

15 In accordance with my invention a film of conducting material is deposited in a good vacuum upon the inner surface of a sealed bulb and good electrical connections with leading-in conductors are provided by 20 means of more conducting localized deposits of metal films adjacent the leading-in conductors. My invention includes both a process and a new article of manufacture.

The novel features of my invention are 25 set forth with particularity in the appended claims. For a better understanding of my invention, reference may be had to the appended drawings taken in connection with the accompanying description.

30 Figure 1 is a sectional view of the resistance unit in the first stage of manufacture; Fig. 2 is a sectional view of the unit provided with localized terminal films at the ends of the inclosing bulb, and Fig. 3 is a sectional view of the completed unit.

As shown in Fig. 1 the unit consists of 35 an elongated bulb 1 consisting of glass, or other suitable non-conducting material. In this bulb is mounted a metal holder 2, one 40 end of which is sealed into the wall of the container 1, and which is specially bent near the sealed-in end to touch the wall of the container for an appreciable part of its length. A filament 3 of molybdenum, tungsten, titanium, or other suitable conducting 45 material is connected at one end to the holder 2 and at the other end to a short leading-in conductor 4, also sealed into the wall of the container 1. Near the ends of the 50 filament 3 are wound short sections 5 and 6 of some material of relatively lower volatility than the filament 3, for example, copper, nickel, silver, or suitable alloys. At the end of the container 1, opposite the end

into which the holder 2 is sealed, there is 55 provided another leading-in conductor 7 sealed into the wall of the container and having a section bent so as to be in close contact with the wall of the container near the end.

With the tube thus assembled a good 60 vacuum is produced in the container, the bulb being heated during exhaustion and the same degree of care being exercised as is good practice in the exhaustion of incandescent lamps. Preferably the highest 65 vacuum attainable with the use of the most efficient pumps such as the condensation pump or the molecular pump, is produced in the bulb.

A heating current is passed through the 70 filament 3 through the holder 2, leading-in wire 4, until the metal bodies 5 and 6 are vaporized by the heat generated in the filaments. The metal vapor is deposited 75 locally at the ends of the bulb 1, as indicated in Fig. 2. The heating current is then increased until the filament itself is more or less volatilized as may be desired. The 80 volatilized metal is deposited by a closely 85 adherent filament upon the surface of the bulb, a good electrical connection being established by its deposition upon the already deposited metal filament at the ends of the bulbs.

By properly proportioning the bulb and 90 adjusting the length of time that the thermal evaporation of the filament is continued and the temperature at which the evaporation is carried on, the thickness of 95 the resistance filament may be easily predetermined. This is not possible in the liquid or paste type of high resistances formerly used. When preparing the conducting film allowance must be made for 100 the temperature coefficient of the deposited film. In practice, the resistance is observed during forming and the deposition is stopped at such point that the film when cooled to room temperatures will 105 have the desired resistance. This precaution is only necessary as the forming temperature with a highly incandescent filament is several hundred degrees above room temperature.

As shown in Fig. 3, the completed unit is 110 preferably provided with conducting caps 8 and 9 contacting with the leading-in con-

ductors 4 and 7, and held in position by a body of cement 10 filling the space between the ends of the tube and terminal caps.

As the described resistances remain at their constant predetermined value during use and do not polarize, they are superior to the various forms of higher resistance now in use.

Although resistance units embodying my invention may be manufactured to have almost any desired resistance, from a few ohms upward, my invention is more particularly applicable to units of small current carrying capacity having resistances somewhere within the range of about 25,000 ohms to 20 megohms.

What I claim as new and desire to secure by Letters Patent of the United States, is:—

1. An electrical resistance unit comprising 20 a sealed non-conducting container, current conductors sealed into said container, a film of refractory conducting material upon the inner surface of said container, and localized films of conducting material contacting both 25 with said conductors and said film.

2. An electrical resistance unit comprising an evacuated glass tube, current conductors sealed into said tube, a film of refractory metal located upon the inner surface of 30 said tube, and areas of good conducting material contacting with said conductors and

said film, at the ends only and with said current conductors.

3. An electrical resistance unit comprising an evacuated glass tube, leading-in conductors sealed into the ends of said tube, a film of molybdenum located upon the inner surface of said tube intermediate said conductors and localized films of copper at the ends of said tube contacting with said 40 molybdenum film and said conductors.

4. An electrical resistance unit comprising a sealed container of insulating material, a gas-free film of conducting material deposited on the inner surface of said container by evaporation in an inclosed space, means for contacting with said film at two separated points and leading in conductors joined to said contacting means.

5. The process of making electrical resistance units which consists in evaporating within an evacuated glass tube and near the ends thereof, a body of metal sufficient in amount to produce a localized film, and then thermally evaporating a filament of refractory metal located to deposit a continuous film of metal upon the inner surface of said tube connecting said first-deposited, localized films of metal.

In witness whereof, I have hereunto set 60 my hand this 5th day of November, 1917.

JOHN H. PAYNE.